# EUROPEAN PATENT APPLICATION

(11) **EP 2 505 697 A1**
(43) Date of publication of application: **03.10.2012**
(21) Application number: 10832568.9
(22) Date of filing: 11.08.2010
(51) Int. Cl.: D01D 5/06, D01D 10/02, D01D 1/02

(54) **METHOD FOR UNIFORMLY PRODUCING FILAMENT FROM ULTRA-HIGH MOLECULAR WEIGHT POLYETHYLENE HIGH-SHEARED SOLUTION**

(30) Priority: 26.11.2009 CN 200910224216
(71) Applicant: Ningbo Dacheng Advanced Material Co., Ltd, Cixi, Zhejiang 315300 (CN)
(72) Inventor: CHEN, Chengsi, Cixi Zhejiang 315300 (CN); XU, Shian, Cixi Zhejiang 315300 (CN); CHEN, Guanjun, Cixi Zhejiang 315300 (CN)
(74) Representative: Brouwer, Hendrik Rogier
(86) International application number: PCT/CN2010/075868
(87) International publication number: WO 2011/063661

(57) **Abstract**

A method for uniformly producing spinning from an ultra-high molecular weight polyethylene high-sheared solution. An ultra-high molecular weight polyethylene is mixed with a solvent in a certain proportion to produce an ultra-high molecular weight polyethylene emulsified solution by high shear, the solution is extruded to spin by a dual-screw extruder, a frozen gel pre-filament is produced by immersion in a freezing water, and then a high strength and high modulus polyethylene fiber is produced by hydrocarbon rinsing, extraction-extension, drying and several times of thermal-extension. The method is low in production energy consumption, is environment friendly, has a short process, and the filament produced by the method has a good mechanical performance and a small fiber deviation.

## Description

### Technical Field

The invention relates to a production method for uniformly producing a two-step process filament from an ultra-high molecular weight polyethylene high-sheared solution.

### Background Technology

In recent years, the research on production of an ultra-high strength and high modulus fiber from a raw material, i.e. ultra-high molecular weight polyethylene has been very active. The two-step process is adopted in the prior art for producing the high modulus fiber: as the first step, intermittent swelling is firstly adopted, that is, the ultra-high molecular weight polyethylene and a solvent are firstly swollen at high temperature in a kettle (heating is generally performed at the temperature from 90 to 120°C, and the heating swelling time is up to 30 to 90 minutes); and as the second step, after extruding and spinning through a dual-screw extruder, a frozen gel filament is quenched, rolled and formed, then the frozen gel filament is extracted by an extraction agent, namely gasoline or carbon tetrachloride, dimethylbenzene, methylene dichloride and the like, and then the production of the fiber is completed through the processes of drying, super multiple thermal drawing and the like.

The filament is generally produced by using the following methods in the prior art:
1. Chinese patent ZL85107352 "Method for Continuously Producing Uniform High Molecular Polymer Solution" discloses a method for producing a high molecular polymer solution. A suspension which is formed by a finely broken high molecular polymer suspending in an appropriate solvent can be produced by the method, and the high molecular polymer solution can be continuously produced at a certain temperature from the high molecular weight polymer through a positive rotation dual-screw extruder equipped with an alternate mixing and conveying part. According to the process, the temperature range for producing the solution is 90°C to 220°C, the heating time is up to 30 to 40 minutes, and the rotational speed of screws is up to 150 to 300 revolutions/minute. It is well known that the melting point of high molecular weight polyethylene is only about 136°C, and great degradation of molecular weight and separation of molecular weight of the high polymer can be seriously affected if heating stays at such a high temperature for 30 to 40 minutes, thereby resulting in low fiber strength and great energy consumption for production.
2. United states patent-US4413110 (Allied) completes the dissolution process by pre-dissolving an ultra-high molecular weight polyethylene in paraffin oil, further re-dissolving it using a dual-screw mixer, and finally feeding the produced slurry into a dual-screw extruder. The purpose of the pre-dissolution in the process is to shorten the residence time of the slurry in the dual-screw extruder, but the pre-dissolution has the problem of thermal oxidative degradation of the polyethylene in process; and furthermore, equipment is complex, and the dual-screw mixer is a high-temperature pressure container that is difficult to manufacture. Allied also introduces a new process in US4784820, a slurry formed by pre-dissolving a ultra-high molecular weight polyethylene in paraffin oil is fed into a high-speed drum mixer (1725 r.p.m) to homogenize the slurry, and the slurry is fed into a single screw under a certain pressure to perform final dissolution so as to produce a polyethylene spinning solution. The process has potential safety hazard in production; and furthermore, the obtained polyethylene spinning solution is poorer in uniformity. Moreover, it is well known that the pressure and the rotational speed of screws are main factors affecting the stability of filament, and low pressure of the screws could further affect the stability of filament.
3. Chinese patent ZL97106768.6 adopts an ultra-high molecular weight polyethylene to perform appropriate swelling in a solvent so as to produce a suspension, and the suspension is continuously and quantitatively fed into a dual-screw extruder under normal pressure for completing the processes of swelling, dissolution, defoaming, metering output and the like so as to continuously produce a uniform spinning solution. The process is intermittent and long in flow. The high molecular weight polyethylene and the solvent are firstly mixed in a reaction kettle, a mixed solution is heated to 90°C to 120°C, heat insulation is performed at this temperature for 10 minutes to 1 hour for swelling so as to produce the suspension, the swollen suspension is placed in another reaction kettle for cooling, and the suspension is quantitatively and continuously fed into the dual-screw extruder for completing the production of a filament after cooling. The process disclosed in the patent is an intermittent kettle type operation process; and furthermore, the concentrations, the temperatures and the particle sizes of the suspensions between the kettles are hardly consistent during the production process, so that the performances of a product are unstable and the whole production process is complex in operation.
4. In the Chinese patent application with the application number 200810034215, a spinning process of an ultra-high molecular weight polyethylene fiber with high strength and high modulus is disclosed, which is a one-step process swelling and dissolution-continuous spinning process. The one-step process has the shortcoming that, as the swelling temperature is higher, the degradation rate of high molecular weight polymer is increased during the swelling process, and accordingly, the mechanical properties of fiber become poorer.
5. Chinese patent with the patent number ZL90102855.X discloses a method for producing a high strength and high modulus polyethylene fiber. In the method, an ultra-high molecular weight polyethylene is firstly dissolved in a kerosene solvent to produce a semi-dilute solution, then the semi-dilute solution is extruded by a dual-screw spinning component, a frozen gel fiber is formed by quenching in a freezing solution (the name of the process is quenching of frozen gel filament), the solvent, namely gasoline, is further utilized to extract kerosene contained in the frozen gel fiber and the fiber is dried, and then super multiple thermal drawing is performed. The process adopts the method in the technology 3, namely, the inter-kettle intermittent heating and swelling process, that is dissolving the ultra-high molecular weight polyethylene in the kerosene solvent to produce the semi-dilute solution, and its shortcomings are also similar to those in the technology 3. As the intermittent kettle type operation process is adopted, non-uniform concentration, temperature and particles of the semi-dilute solution between the kettles during the production process are caused, thermal oxidative degradation of molecular weight of a high molecular polymer are also caused, and the mechanical properties of fiber are further affected. In addition, the kerosene is adopted as the solvent in the method; because the kerosene is volatile and flammable, the kerosene is easy to volatilize and be mixed with air to form an explosive mixed gas under the actions of long-term heating and stirring, thus great hidden trouble is caused to safety production; furthermore, the kerosene is stinky slightly, which is liable to cause air pollution and quite harmful to health of operator.
6. Chinese patent ZL03106030.7 discloses a method for producing a high strength polyethylene fiber, which is: a polymer mixture is dissolving in a solvent to enable the concentration to be more than 5wt% and less than 89wt%, then spinning and drawing. Said mixture is formed by 99 parts by weight to 50 parts by weight of a high molecular weight polymer (A) mainly containing an ethylene component with the limiting viscosity number [η] above 5 and the ratio of weight average molecular weight to number average molecular weight (Mw/Mn) below 4, and 1 part by weight to 50 parts by weight of an ultra-high molecular weight polymer (B) at least with the limiting viscosity number 1.2 times as much as that of the high molecular weight polymer (A).

The pre-dissolution or pre-swelling step exists in each of Chinese patents ZL85107352, ZL97106768.6 and United states patent -US4413110 (Allied), then the production of the ultra-high molecular weight polyethylene solution is completed by further dissolution through screws. The process is intermittent actually, so low production efficiency, high energy consumption, complex equipment structure and long time required for production during the whole production process, thermal oxidative degradation of the ultra-high molecular weight polyethylene in the production process and other defects are inevitable, and the solution produced by the above method is further non-homogeneous.

In summary, the conventional two-step process production method in the prior art has the following shortcomings: 1) When the ultra-high molecular weight polyethylene and the solvent are mixed for swelling, thermal oxidative degradation of the ultra-high molecular weight polyethylene can be caused due to high swelling reaction temperature and long swelling time, thus the mechanical properties of fiber are reduced. 2) Containers adopted during the intermittent swelling process include a plurality of swelling kettles, and the reaction temperature, the solution concentration and the granularity in the solution in each swelling kettle participating the reaction during the swelling process are different, so that the performances of the fibers produced in subsequent processes are greatly different. 3) The solution in each swelling kettle is swollen and then sent to the dual-screw extruder via a vacuum pump for extrusion and spinning, and then the frozen gel filament is quenched, rolled and formed. The shrinkage of the frozen gel as-spun fiber is non-uniform due to the differences in the solution concentration, the granularity, the temperature and the like between the kettles. 4) The non-uniform shrinkage of the frozen gel as-spun fiber is caused by the defects in the previous processes. Then, the frozen gel as-spun fiber is subjected to the extraction process, and in this process, gasoline, carbon tetrachloride, dimethylbenzene, methylene dichloride and the like are generally used as extraction agents, the processes of drying and super multiple thermal drawing are further performed to obtain the fiber having broken filament, roller winding and other phenomena, that result in the defects of low mechanical properties and poor uniformity in the fiber; in addition, as the used extraction agents are all flammable and explosive liquids and very volatile, the shortcomings of great potential safety hazard, poor production environment, great consumption of energy and the like are further caused during the extraction process.

### Contents of Invention:

The production of an ultra-high molecular weight polyethylene uniform spinning solution is one of the key points for producing a polyethylene frozen gel filament and can directly affect the spinnability of an ultra-high molecular weight polyethylene filament, as well as quality uniformity, mechanical properties, energy conservation, consumption reduction and other important factors of the resultant fiber. The invention adopts high shear to enable the spinning solution, obtained from an ultra-high molecular weight polyethylene and a solvent by grinding under normal temperature, to be uniform in quality; and due to the adoption of a normal temperature treatment method, oxidative degradation of molecular weight of the ultra-high molecular weight polyethylene is avoided. The process requirements of ultra-high molecular weight polyethylene fibers in different specifications and high drawing ratio can be met, the phenomena of roller winding by filament, filament breakage, broken filament and non-uniform denier caused by own poor quality of the solution can be greatly reduced, therefore, a key role can be played in stabilizing the production of the filament and greatly improving the mechanical properties of the fiber.

In view of the defects existed in the prior art, the invention provides a method for uniformly producing a filament from an ultra-high molecular weight polyethylene high-sheared solution, and the problems existed in the prior production processes can be basically avoided by using the method; furthermore, the method provided by the invention is short in processing time, and degradation of the ultra-high molecular weight polyethylene seldom occurs during the processing process.

The method for uniformly producing the filament from the ultra-high molecular weight polyethylene high-sheared solution in the invention comprises the following steps: selecting an appropriate solvent and an ultra-high molecular weight polyethylene, continuously conveying the solvent and the high molecular weight polyethylene into a mixer for stirring at normal temperature in a certain proportion according to the process requirements in an automatic metering way so as to produce a uniform suspension, connecting the uniform suspension to a high shear pump through a pipeline, grinding the ultra-high molecular weight polyethylene in the solvent in a circulating and high-speed manner through high-speed operation of the high shear pump, and finally, obtaining the uniform milky spinning solution and continuously feeding the uniform milky spinning solution into a dual-screw extruder for spinning.

The operations above are performed in an automatic, metering and continuous manner, and the output flow rate and the input flow rate of the solution are kept consistent. The structure in the high shear pump is compact, and the ultra-high molecular weight polyethylene is highly and uniformly emulsified in the solvent under high-speed grinding. Although the high shear pump operates at high speed during the production process, all the processes are performed at normal temperature; furthermore, the solvent is taken as a cooling medium in the high shear pump, and a cooling device is further arranged outside the high shear pump, so that high-speed grinding hardly leads to the increase of the temperature of the solution; moreover, the grinding is completed within a very short period of time and heating is not required in the whole working process, so the problem of degradation of the ultra-high molecular weight polyethylene or separation of molecules caused by high temperature can be avoided during the production process.

By using the method of the invention, the ultra-high molecular weight polyethylene solution can be highly homogenized and emulsified, and both the low-concentration high molecular polyethylene solution and the high-concentration high molecular polyethylene solution can be produced. Furthermore, processing is performed at normal temperature, and heating is not required to further reduce energy consumption greatly; and the high shear pump is connected with the dual-screw extruder by the pipeline, single high shear pump or the plurality of high shear pumps which are connected in series or parallel can operate simultaneously according to the actual production needs, therefore, the production efficiency can be greatly improved and the production cost can be reduced. The method of the invention is a brand new production method which is totally different from the existing reported technologies; and the ultra-high molecular weight polyethylene solution which is highly homogenized and emulsified and produced by utilizing the method can meet the production requirements of the ultra-high molecular weight polyethylene fibers in different specifications, the phenomena of roller winding by filament, filament breakage, broken filament, non-uniform denier and the like caused by own poor quality of the solution can be greatly reduced, and a key role can be played in improving the mechanical properties of fiber.

The specific steps of the method of the invention are as follows:

### The first step:

1.1 selecting the ultra-high molecular weight polyethylene and selecting hydrogenated naphthalene or alkanes as the solvent;
1.2 conveying the ultra-high molecular weight polyethylene into the kettle type stirring mixer in the automatic metering way, simultaneously conveying the solvent into the kettle type stirring mixer in an automatic metering way, and continuously mixing at normal temperature to form the uniform suspension, wherein the mixing ratio is that the weight percent of the ultra-high molecular weight polyethylene is 5 to 20% and the weight percent of the solvent is 80 to 95%, and the mixture ratio between the two, namely the ultra-high molecular weight polyethylene and the solvent, can be adjusted according to the specification of the fiber to be produced;
1.3 conveying the mixed suspension into the high shear pump through the pipeline, enabling the ultra-high molecular weight polyethylene to circulate and be ground at high speed in the solvent through high-speed operation of the high shear pump so as to obtain the homogenized high-sheared ultra-high molecular weight milky spinning solution, and then continuously conveying the milky spinning solution into the dual-screw extruder through the pipeline;
1.4 enabling the high-sheared ultra-high molecular weight milky spinning solution to complete heating swelling, mixing and dissolution of the ultra-high molecular weight polyethylene in the pipeline dual-screw extruder, and extruding into a spinning component for spinning via a thread element, wherein the process step is mainly divided into three sections: the first section is heating and swelling the ultra-high molecular weight polyethylene homogenized spinning milky solution; the second section is reheating, mixing and dissolving through the thread element; and the third section is further performing heat insulation and metering and conveying to the spinning component through the thread element;
1.5 directly quenching an ultra-high molecular weight as-spun filament extruded to spin by the dual-screw extruder in a freezing water so as to get a frozen gel pre-filament;
1.6 firstly performing pre-drawing on the frozen gel filament, and then performing extraction drawing, wherein the extraction adopts a closed reverse drawing process, and a hydrocarbon type environment-friendly cleaning agent is selected as an extraction agent; further performing secondary pre-drawing, wherein the secondary pre-drawing is different from the extraction drawing and specially is dry process normal temperature direct drawing; and
1.7 drying and rolling the fiber after the operation process in the step 1.6.

The above-mentioned step is the first step (a first unit) of the two-step process spinning method of the invention. Then, the second step is performed (a second unit):
2.1 firstly performing swelling rate preheating on a rolled multifilament obtained in the first step of the two-step production process, and further drawing with three-passage hot air; and
2.2 performing thermal shaping, fiber surface treatment and natural cooling on the fiber subjected to three-passage thermal drawing, and rolling a finished product.

The invention is the method for producing the two-step process filament by high shear and uniform swelling of the ultra-high molecular weight polyethylene, and the filament produced through the method has the advantages of high mechanical properties of fiber, small fiber deviation, low energy consumption for production, good production environment, short production process flow and the like.

### Modes for Carrying Out the Invention

In combination of the following embodiments, the invention will be further described in details.

The specific implementation steps of the method of the invention are as follows:

### The first step:

1.1 selecting an ultra-high molecular weight polyethylene with the molecular weight of 1 to 5 millions, and selecting naphthalene or alkanes, such as paraffin oil, tetraline or white oil type mineral oil as a solvent (the mineral limiting viscosity is 5 to 80#);
1.2 conveying the ultra-high molecular weight polyethylene into a kettle type stirring mixer in an automatic metering way, simultaneously conveying the solvent into the kettle type stirring mixer in an automatic metering way for mixing, and continuously mixing at normal temperature to form a uniform suspension, wherein the mixing ratio is that the weight percent of the ultra-high molecular weight polyethylene is 5 to 20% and the weight percent of the solvent is 80 to 95%, and the mixture ratio can be adjusted according to the specification of fiber;
1.3 conveying the mixed ultra-high molecular weight polyethylene suspension into a high shear pump through a pipeline, enabling the ultra-high molecular weight polyethylene in the mixed suspension to circulate and be ground at high speed in the solvent through high-speed operation of the high shear pump so as to obtain a homogenized high-sheared ultra-high molecular weight milky spinning solution, and then continuously conveying the milky spinning solution into a dual-screw extruder through the pipeline; wherein the working flow rate of the high shear pump can be adjusted between 10m3/h and 500m3/h according to the process requirements;
1.4 continuously feeding the high-sheared ultra-high molecular weight milky spinning solution into the dual-screw extruder through the pipeline, then completing heating swelling, mixing, dissolution and other processes of the ultra-high molecular weight polyethylene in the dual-screw extruder, and extruding into a spinning component for spinning via a thread element, wherein the length/diameter ratio of double screws is 1: 50, and the operation speed of the double screws is 120-300 revolutions/minute; and the process in the dual-screw extruder is mainly divided into three sections: the first section is heating and swelling the ultra-high molecular weight polyethylene homogenized spinning milky solution, wherein the swelling temperature is 70°C to 110°C (increasing along with the speed of the double screws); the second section is reheating, mixing and dissolving through the thread element, wherein the temperature for mixing and dissolving is 130°C to 220°C (increasing along with the speed of the double screws); and the third section is further performing heat insulation and metering and conveying to the spinning component through the thread element, wherein the temperature for heat insulation and conveying is 200°C to 220°C;
1.5 directly quenching an ultra-high molecular weight as-spun filament extruded to spin by the dual-screw extruder in a freezing water at the temperature of 0°C to 5°C so as to get a frozen gel pre-filament (called as frozen gel filament generally), wherein the diameter of the as-spun monofilament is 1 to 1.5mm, the linear speed of quenching is 1 to 5m/min, and the residence time of quenching is 30 seconds to 100 seconds;
1.6 firstly pre-drawing the frozen gel filament by 1-5 times, further extracting, and then redrawing by 2-8 times, wherein the extraction adopts a closed reverse drawing process, a hydrocarbon type environment-friendly cleaning agent is selected as an extraction agent, the cleaning agent may be trifluorotrichloroethane, trichloroethane or dichloroethane, etc., the hydrocarbon type environment-friendly cleaning agent can be not only volatilized naturally but also recycled, and the recycling rate can reach 95%; further performing secondary pre-drawing, wherein the secondary pre-drawing is different from the extraction drawing and specially is dry process normal temperature direct drawing; and
1.7 drying and rolling the fiber after the operation process in the step 1.6, wherein the drying temperature is 40°C to 60°C, the drying time is 10 to 40 minutes, and a product after drying and rolling is generally called as an ultra-high molecular weight polyethylene multifilament.

The above-mentioned step is the first step of the two-step process spinning method of the invention, and then the second step is performed:
2.1 firstly performing swelling rate preheating on the rolled multifilament produced in the first step of the two-step process production process at the temperature of 40°C to 60°C, wherein the preheating residence time is 20 to 30 minutes; and then continuously drawing with three-passage hot air, wherein the first passage drawing is of 2-4 times, and the circulating temperature of the hot air is 110°C to 140°C; the second passage drawing is 1.5 to 2.5 times after the first drawing, and the circulating temperature of the hot air is 130°C to 145°C; the third passage drawing is 0.5 to 1.5 times after the second drawing, and the circulating temperature of the hot air is 130°C to 165°C; and an ultra-high molecular weight polyethylene molecular chain can be fully extended after drawing with the three-passage hot air, molecular crystals are uniformly arranged, excellent mechanical properties can be obtained, and the strength is not less than 40g/D; and
2.2 then performing thermal shaping at the temperature of 130°C to 150°C on the fiber subjected to three-passage thermal drawing , performing surface treatment on the fiber, then naturally cooling and rolling a finished product, wherein the linear speed of thermal shaping is 15-50m/min and plasma corona or glow surface treatment is simultaneously continuously performed during the process.

## Claims

1. A method for uniformly producing a filament from an ultra-high molecular weight polyethylene high-sheared solution, which is specifically as follows: selecting an appropriate solvent and an ultra-high molecular weight polyethylene, continuously conveying the solvent and the high molecular weight polyethylene into a mixer for stirring at normal temperature in a certain proportion according to the process requirements in an automatic metering way so as to produce a uniform suspension, connecting the uniform suspension to a high shear pump through a pipeline, grinding the ultra-high molecular weight polyethylene in the solvent in a circulating and high-speed manner through high-speed operation of the high shear pump, and finally, obtaining a uniform milky spinning solution and continuously feeding the uniform milky spinning solution into a dual-screw extruder for spinning.

2. The method according to claim 1, **characterized in that** the method specifically comprises the following two steps:
the first step:
1.1 selecting the ultra-high molecular weight polyethylene and selecting hydrogenated naphthalene or alkanes as the solvent;
1.2 conveying the ultra-high molecular weight polyethylene into a kettle type stirring mixer in an automatic metering way, simultaneously conveying the solvent into the kettle type stirring mixer in an automatic metering way for mixing, and continuously mixing at normal temperature to form a uniform suspension;
1.3 conveying the mixed suspension into the high shear pump through a pipeline, enabling the ultra-high molecular weight polyethylene in the mixed suspension to circulate and be ground at high speed in the solvent through high-speed operation of the high shear pump so as to obtain the homogenized high-sheared ultra-high molecular weight milky spinning solution, and then continuously conveying the milky spinning solution into the dual-screw extruder through the pipeline;
1.4 enabling the high-sheared ultra-high molecular weight milky spinning solution to complete heating swelling, mixing and dissolution of the ultra-high molecular weight polyethylene in the pipeline dual-screw extruder, and extruding into a spinning component for spinning via a thread element, wherein the process step is mainly divided into three sections: the first section is heating and swelling the ultra-high molecular weight polyethylene homogenized spinning milky solution; the second section is reheating, mixing and dissolving through the thread element; and the third section is further performing heat insulation and metering and conveying to the spinning component through the thread element;
1.5 directly quenching an ultra-high molecular weight as-spun filament extruded to spin by the dual-screw extruder in a freezing water so as to get a frozen gel pre-filament;
1.6 firstly performing pre-drawing on the frozen gel filament, and then performing extraction drawing, wherein the extraction adopts a closed reverse drawing process, and a hydrocarbon type environment-friendly cleaning agent is selected as an extraction agent; further performing secondary pre-drawing, wherein the secondary pre-drawing is different from the extraction drawing and specifically is dry process normal temperature direct drawing; and
1.7 drying and rolling the fiber after the operation process in the step 1.6;
and the second step:
2.1 firstly performing swelling rate preheating on a rolled multifilament obtained in the first step, and further drawing with three-passage hot air; and
2.2 performing thermal shaping, fiber surface treatment and natural cooling on the fiber subjected to three-passage thermal drawing, and rolling a finished product.

3. The method according to claim 2, **characterized in that**,
in the step 1.1, the solvent is paraffin oil, tetraline or white oil type mineral oil;
in the step 1.2, the mixing ratio is that the weight percent of the ultra-high molecular weight polyethylene is 5-20% and the weight percent of the solvent is 80-95%, and the mixture ratio can be adjusted according to fiber specification;
in the step 1.3, the working flow rate of the high shear pump is 10m3/h to 500m3/h;
in the step 1.4, the length/diameter ratio of double screws is 1: 50, the operation speed of the double screws is 120 to 300 revolutions/minute, the temperature for heating and swelling the ultra-high molecular weight polyethylene homogenized spinning milky solution in the first section is 70°C to 110°C, the temperature for mixing and dissolving in the second section is 130°C to 220°C and the temperature for heat insulation and conveying in the third section is 200°C to 220°C;
in the step 1.5, the diameter of the as-spun monofilament is 1-1.5mm, the frozen gel pre-filament (called as frozen gel filament generally) is obtained by directly quenching the as-spun monofilament in the freezing water at the temperature of 0°C to 5°C, the linear speed of quenching is 1 to 5m/min, and the residence time of quenching is 30 seconds to 100 seconds;
in the step 1.6, the frozen gel filament is firstly pre-drawn by 1-5 times, further extracted and then drawn by 2-8 times, the extraction adopts a closed reverse drawing process, a hydrocarbon type environment-friendly cleaning agent is selected as an extraction agent, and the cleaning agent may be trifluorotrichloroethane, trichloroethane or dichloroethane; and
in the step 1.7, the drying temperature for drying and rolling is 40°C to 60°C, and the drying time is 10 to 40 minutes.

4. The method according to claim 2, **characterized in that**,
in the step 2.1, the swelling rate preheating is firstly performed at the temperature of 40°C to 60°C on the rolled multifilament obtained in the first step, the preheating residence time is 20 to 30 minutes, then drawing with the three-passage hot air is further continuously performed, the first passage drawing is of 2-4 times, the circulating temperature of the hot air is 110°C to 140°C, the second passage drawing is 1.5 to 2.5 times after the first drawing, the circulating temperature of the hot air is 130°C to 145°C, the third passage drawing is 0.5-1.5 times after the second drawing, the circulating temperature of the hot air is 130°C to 165°C, and an ultra-high molecular weight polyethylene molecular chain can be fully extended, and molecular crystals are uniformly arranged; and
in the step 2.2, thermal shaping is further performed at the temperature of 130°C to 150°C on the fiber subjected to three-passage thermal drawing, and the linear speed of thermal shaping is 15 to 50m/min.

5. The method according to claim 4, **characterized in that**, in the step 2.2, plasma corona or glow surface treatment is simultaneously continuously performed during the processes of thermal shaping, surface treatment and natural cooling of the fiber.
